

No. 658,483.

Patented Sept. 25, 1900.

C. J. COLEMAN.

PROCESS OF OXIDIZING NEGATIVE ELECTRODES FOR PRIMARY BATTERIES.

(Application filed Dec. 20, 1899.)

(No Model.)



Witnesses

G. S. Elliott.  
J. Henry Kaiser -

Inventor:

Clyde J. Coleman,

by Robert Burns

Attorney

# UNITED STATES PATENT OFFICE.

CLYDE J. COLEMAN, OF CHICAGO, ILLINOIS, ASSIGNOR TO THOMAS J. RYAN,  
OF NEW YORK, N. Y.

## PROCESS OF OXIDIZING NEGATIVE ELECTRODES FOR PRIMARY BATTERIES.

SPECIFICATION forming part of Letters Patent No. 658,483, dated September 25, 1900.

Application filed December 20, 1899. Serial No. 741,030. (No specimens.)

To all whom it may concern:

Be it known that I, CLYDE J. COLEMAN, a citizen of the United States, and a resident of Chicago, in the county of Cook and State of Illinois, have invented certain new and useful Improvements in Processes of Oxidizing Negative Electrodes for Primary Batteries; and I do hereby declare the following to be a full, clear, and exact description of the same, reference being had to the accompanying drawing, forming a part of this specification.

This invention relates to the manufacture of negative electrodes for primary batteries, and more especially to that type of such negative electrodes which are composed, mainly, of copper oxid.

The object of the present improvement is to provide a simple and efficient process of oxidizing such copper oxid electrodes and in which a very perfect agglomeration of the oxid upon the holding support or casing is effected coincident with the process of oxidation to produce a negative electrode that is free from the usual cracks or seams and the consequent inert portions, bad contacts, and high resistances. Accordingly the present process comprises the filling or coating of the holding casing or support with finely-divided or porous metallic copper in any usual and approved manner and the conversion of such filling or coating of metallic copper into an active oxid of copper by a continued exposure to an oxidizing atmosphere in the presence of moisture until such filling or coating is wholly converted into an oxid. In like manner the present process involves the reoxidation of negative battery electrodes in which the active copper oxid has been reduced to metallic copper by previous use in a battery.

In the accompanying drawing, illustrative of the present invention, an apparatus is shown adapted to treat a number of negative electrodes at one time.

Referring to the drawing, 1 represents a closed chamber, in the bottom portion of which is contained a layer of water adapted to afford the requisite moisture required in the present process.

2 is a supporting partition or diaphragm, upon which the series of electrodes 3 are supported in any suitable manner.

4 is the air-inlet duct connected to the chamber 1 at a point below the partition 2 and immediately above the layer of water; 5, an air-

outlet duct arranged near the upper end of 55 the chamber.

6 is a heating jet or burner arranged beneath the air-inlet duct 4 and adapted to heat the incoming air to the desired degree of temperature.

7 is the water-supply pipe, and 8 the drain-pipe, by means of which a constant and predetermined amount of water is maintained in the bottom portion of the chamber.

In use the heating jet or burner 6 will maintain the desired degree of circulation of air through the oxidizing-chamber 1; but in some cases, and more especially when such heating effect is dispensed with, the circulation of air through the chamber will be effected in a positive manner by any usual well-known means. With the present process the oxidation of the copper takes place in a rapid and uniform manner and depends more upon the action of the moisture contained in the air passing through the oxidizing-chamber, as but a very moderate heat is employed. As a result of such uniform oxidation of the present process, the usual checking and cracking of the oxid coating or filling is avoided.

Having thus fully described my said invention, what I claim as new, and desire to secure by Letters Patent, is—

1. The herein-described process of oxidizing negative electrodes for primary batteries, the same comprising the oxidation of a body of finely-divided or porous copper into a coherent mass by placing it in an oxidizing atmosphere and simultaneously supplying to it a requisite amount of moisture and controlling 85 the supply of moisture, substantially as set forth.

2. The herein-described process of oxidizing negative electrodes for primary batteries, the same comprising the oxidation of a body of finely-divided or porous copper into a coherent mass, by placing it in an oxidizing atmosphere and simultaneously supplying to it the requisite amount of moisture and the required degree of temperature above normal, and controlling the supply of moisture and temperature, substantially as set forth.

Signed by me at Washington, District of Columbia, this 11th day of December, 1899.

CLYDE J. COLEMAN.

Witnesses:

ROBERT BURNS,  
M. H. HOLMES.